

# UNITED STATES PATENT OFFICE.

BAT SMITH, OF SPANISH CAMP, TEXAS.

## COMPOSITION FOR PRESERVING WOOD.

SPECIFICATION forming part of Letters Patent No. 244,327, dated July 12, 1881.

Application filed April 21, 1881. (No specimens.)

*To all whom it may concern:*

Be it known that I, BAT SMITH, of Spanish Camp, in the county of Wharton and State of Texas, have invented a new and Improved Compound for Preserving Wood, of which the following is a specification.

My composition consists of the following ingredients, combined in the proportions stated—  
viz., coal-tar, eight parts; crude carbolic acid, one part; crude pyroligneous acid, three-fourths part. The crude carbolic acid and the crude pyroligneous acid are first thoroughly mixed, and this mixture is added to the coal-tar, and the whole is then again thoroughly mixed. This compound is gently heated, but is not permitted to boil.

The wood to be treated is placed in some suitable vessel which is filled with the compound, so that the wood is completely immersed in the same. The wood remains in this compound until it is completely saturated.

The above-described compound can also be used to paint wood with.

The compound is to be used to preserve all kinds of wood, in or above the ground, but is especially adapted for preserving wood in salt water from the ravages of worms, barnacles, &c., and will be found to be of great service for ships' bottoms, piles, caissons, piers, &c.

Having thus fully described my invention, I claim as new and desire to secure by Letters Patent—

The within-described compound for preserving wood, consisting of coal-tar, crude carbolic acid, and crude pyroligneous acid, in the proportions specified.

BAT SMITH.

Witnesses:

L. D. BROWNE,  
H. H. WICKLING.